

Patented Sept. 4, 1934

1,972,760

# UNITED STATES PATENT OFFICE

1,972,760

## GUM INHIBITOR FOR HYDROCARBON FUELS

William S. Calcott, Penns Grove, N. J., and Ira E. Lee, Wilmington, Del., assignors, by means assignments, to Gasoline Antioxidant Company, Wilmington, Del., a corporation of Delaware

No Drawing. Application August 23, 1929,  
Serial No. 333,633

19 Claims. (Cl. 44—8)

This invention relates to improvement in means for the protection of liquid hydrocarbon products against discoloration and formation of insoluble and gummy products, and more particularly to improved materials for use with unsaturated liquid hydrocarbons which may be used as fuels.

Liquid hydrocarbons as commercially produced, particularly when prepared by the distillation or cracking of petroleum, possess a tendency to discolor on standing and to form gums and resinous substances. Gasolines produced by the modern cracking processes are extremely complicated mixtures comprising many constituents, the character of these constituents and the relative proportions of different constituents depending upon the source of the crude and the particular cracking process employed. Besides the normal and branched chain paraffines, there are often present substantial percentages of aromatic hydrocarbons. The crude cracked gasoline always contains unsaturated hydrocarbons, such for example as olefines and diolefines. Although there may be present some compounds containing a triple bond, these are probably not compounds such as may be formed by the polymerization of acetylene, but rather such compounds as may be formed by the isomerization of dienes and having the general formula  $C_nH_m$  where  $m$  is greater than  $n$ , but less than  $2n+2$ . These unsaturated compounds in the presence of air are capable of oxidation to form a series of products, some of which are resinous or gummy. The diolefines, and more unsaturated hydrocarbons, are particularly easily oxidized. Differences in structure other than the degree of unsaturation cause considerable variation in the tendency to oxidize, but in general the ease of oxidation increases with the degree of unsaturation. The more recent pressure methods of vapor phase cracking result in a considerably higher percentage of diolefines than the older methods, and it has been stated that these products may run as high as 8 to 15% in unrefined gasoline.

It has been necessary to treat the crude products resulting from the more recent cracking processes in some manner to remove the greater part of these more highly unsaturated products. Among these methods of treatment may be mentioned the sulfuric acid treatment and the fuller's earth vapor phase treatment. While these methods of purification may remove the greater part of the highly unsaturated compounds, it is found that many brands of gasoline tend to discolor on storage and to form a certain amount of gum. The gum appears to be a complex mix-

ture of polymerized hydrocarbons, resins, acids, aldehydes, ketones and peroxides. Its formation is distinctly detrimental in all cases. For example, the deposition of gum in gasoline gives a sticky substance which deposits upon the walls and bottom of the container, and which may cause serious trouble if formed or deposited in the fuel system of internal combustion engines. The soluble portion of the gum is also objectionable because of the introduction of a non-volatile component into the gasoline.

Our invention has for an object the inhibition of the formation of these insoluble gums and resins, with an attendant improvement in the quality of the hydrocarbon and freedom from the difficulties introduced by the formation of the more or less insoluble and sticky, gummy material, such as irregular flow in the fuel and lubricating systems of internal combustion engines. A further object is to make it possible to use as an internal combustion fuel, liquid hydrocarbons such as gasoline, that contain larger amounts of highly unsaturated compounds than commercially used at present. A product of this sort can be produced at a lower cost, and possesses in certain cases, improved anti-knock properties.

We have found that by treating hydrocarbon fuels such as gasoline, and specifically cracked gasoline or gasoline which has a tendency to form gum, the gum formation can be very appreciably inhibited if the hydrocarbon fuel is treated with a diaryl guanidine. More specifically, our invention relates to the use as gum inhibitors for hydrocarbon fuels of compounds of the type represented by



in which R is an aryl group and R' is an aryl group which may be the same as or different from R, and in which both R and R' may contain alkyl substituents.

By way of illustration of our invention, if to a gasoline which undergoes rapid discoloration and gives rise to gum formation upon exposure to sunlight, a small amount of diphenyl guanidine or diorthotolyl guanidine is added, the aging qualities of the gasoline will be substantially improved. We have, for example, stored gasoline for a period of many months—one sample without any inhibitor—the other containing a very small percentage of diorthotolyl guanidine. After a few months storage in the light, the sample without

an inhibitor developed much color and contained a large amount of gum. The sample protected by the diorthotolyl guanidine, on the other hand, developed no color and showed little, if any, increase in the amount of dissolved gum. It will be understood that the example given above has been given merely for the purpose of illustrating our invention, and that we do not wish to be restricted to the specific guanidine or gasoline set forth in the example.

We have discovered that the diaryl guanidines as a class are very effective inhibitors of the gum formation in hydrocarbon fuels. We have tested many of these compounds over prolonged periods, and found them to be effective in the prevention of gum formation even when the hydrocarbon fuel has been exposed to direct sunlight. Some of the substances which we have found to be effective inhibitors are: diphenyl guanidine, di-orthotolyl guanidine, di-para-tolyl-guanidine, di-xylyl-guanidine and phenyl-tolyl-guanidine.

In some cases it has been found advisable to use a mixture of guanidine rather than a single pure product. It has been found in some cases that a combination of two different guanidines is superior in its effect on gasoline to either guanidine used singly.

We may use higher or lower concentrations of any members of the class of compounds represented by the general formula given hereabove, and to secure marked inhibition of gum formation although, of course, the degree of inhibition will vary depending upon the individual guanidine, the concentration of guanidine employed, and the nature of the hydrocarbon fuel. In general, amounts of from 0.0001 of 1% to 0.05 of 1% of inhibitor will be found sufficient for the grades of gasoline at present on the market. It will be obvious, of course, that these percentages may be varied within wide limits. Obviously, our invention is of great importance in freeing internal combustion engines from the annoyance and improper functioning due to the deposition of gum in the fuel system and explosion chamber.

As many apparently widely different embodiments of this invention may be made without departing from the spirit thereof, it is to be understood that we do not limit ourselves to the foregoing examples or descriptions except as indicated in the following patent claims:

We claim:

1. A motor fuel comprising cracked gasoline normally tending to form gum containing, as a gum inhibitor, a small amount of a substance of the type:



in which R is an aryl group and R' is an aryl group which may be the same as R.

2. Gasoline produced by the cracking of petroleum oils containing, as a gum inhibitor, a small amount of a substance of the type:



in which R is an aryl group and R' is an aryl group which may be the same as R.

3. A motor fuel comprising cracked gasoline normally tending to form gum containing, as a

gum inhibitor, a small amount of a substance of the type



80

in which R and R' represent aryl groups at least one of which contains an alkyl group substituted therein.

4. A motor fuel comprising cracked gasoline normally tending to form gum containing, as a gum inhibitor, a small amount of a substance of the type



90

in which R and R' represent alkyl substituted aryl groups.

5. A motor fuel comprising cracked gasoline normally tending to form gum containing, as a gum inhibitor, a small amount of a substance of the type



100

in which R and R' represent aryl groups which may contain substituted alkyl groups.

6. A motor fuel comprising cracked hydrocarbon distillates normally tending to form gum on storage and containing, as a gum inhibitor, a small amount of a substance having the general formula



115

wherein R and R<sub>1</sub> represent aryl groups at least one of which contains an alkyl group substituted therein.

7. A motor fuel comprising cracked hydrocarbon distillates normally tending to deteriorate and form gum on storage and containing, as a gum inhibitor, a small amount of a substance having the following general formula



125

wherein R represents an aryl group and R<sub>1</sub> represents an aryl group which may be the same as R.

8. A motor fuel comprising cracked hydrocarbon distillates normally tending to form gum and containing, as a gum inhibitor, a small quantity of a substance having the following general formula



135

wherein R and R<sub>1</sub> represent phenyl groups at least one of which contains an alkyl group substituted therein.

9. A motor fuel comprising cracked gasoline obtained by vapor phase conversion of high boiling hydrocarbons, normally tending to deteriorate and form gum, and containing as a gum inhibitor a small proportion of a diaryl guanidine.

10. A motor fuel comprising cracked hydrocarbon distillates normally tending to form gum and

150

- containing, as a gum inhibitor, a small amount of di-para-tolyl guanidine. 16. A cracked, highly unsaturated hydrocarbon motor fuel distillate of less-readily detonating type normally tending to develop gum forming constituents, containing diphenylguanidine in quantity sufficient to prevent development of substantial quantities of such gum forming constituents. 80
11. A motor fuel comprising cracked gasoline normally tending to deteriorate and form gum and containing, as a gum inhibitor, a small amount of di-para-tolyl guanidine. 12. A cracked hydrocarbon distillate containing high percentages of unsaturated compounds combined with a gum inhibitor in the form of 10 diphenylguanidine. 85
13. A cracked hydrocarbon motor fuel containing diphenylguanidine in quantities sufficient to inhibit the formation of gums in said fuel. 14. A cracked hydrocarbon distillate having substantially the boiling range of ordinary gasoline and having added thereto a gum inhibitor in the form of a compound containing diphenylguanidine. 90
15. The method of treating cracked petroleum 20 distillates obtained by vapor phase conversion of high boiling hydrocarbons, which consists in adding to such distillates a compound containing diphenylguanidine in quantities sufficient to inhibit the natural evolution of resinous compounds of such distillates. 95

17. The method of stabilizing the characteristics of a cracked, unsaturated hydrocarbon motor fuel distillate of the less-readily detonating type, normally tending to deteriorate and develop gum-forming constituents, which comprises adding thereto prior to such deterioration a small proportion of diphenylguanidine, sufficient to substantially inhibit further gum formation in said distillate.

18. A motor fuel comprising cracked gasoline normally tending to form gum containing, as a gum inhibitor, a small amount of di-ortho-tolyl guanidine. 95

19. Gasoline produced by the cracking of petroleum oils containing, as a gum inhibitor, a small amount of di-ortho-tolyl guanidine.

WILLIAM S. CALCOTT.

IRA E. LEE.

100

30 105

35 110

40 115

45 120

50 125

55 130

60 135

65 140

70 145

75 150